

T. A. BLAKELY.  
Ordnance.

No. 41,662.

Patented Feb. 16, 1864



Witnesses.

C. C. English  
J. L. Combs

Inventor

T. A. Blakeley  
Inventor  
of this art

# UNITED STATES PATENT OFFICE.

THEOPHILUS A. BLAKELY, OF LONDON, ENGLAND.

## IMPROVEMENT IN ORDNANCE.

Specification forming part of Letters Patent No. 41,662, dated February 16, 1864.

*To all whom it may concern:*

Be it known that I, THEOPHILUS ALEXANDER BLAKELY, of Montpelier Square London, England, late captain Royal Artillery, have invented Improvements in Ordnance; and I do hereby declare that the following is a full and exact description thereof.

The inside of a tube being more stretched by pressure from within than the middle and outside, in about the ratio of the squares of the diameters of the layers, I patented in Great Britain, in February, 1855, a method of obtaining increased strength in ordnance by building cannon of two or more concentric tubes, of which the outer compresses the inner to a definite degree, so that on the gun being fired all the concentric tubes act together in resisting the strain. This method has been much used, particularly in America, by Mr. Parrott. Another method of increasing the strength of cannon has been used by the Dutch, and proposed in England by Captain Palliser. It consists in placing a very yielding material—such as bronze or wrought-iron—inside of cast-iron, without any compression of the inner tubes or extension of the outer. This latter plan is not applicable for large ordnance of great power, because metals cannot be found possessing both sufficient difference of extensibility and at the same time the other qualities required for ordnance. I therefore make cannon in the following manner: I build the gun of concentric tubes, the inner tube being of a material that is most extensible within the elastic limit, the next tube less extensible within the elastic limit, and so on, decreasing in extensibility within the elastic limit to the outside. I do not, however, merely fit the tubes together, but I put on each successive layer with so much initial tension that the whole shall be worked by pressure from within to about the same degree—that is to say, the initial tension of the successive tubes shall compensate for any deficiency in the extensibility of the tubes within them, so that all the tubes shall contribute equally of their strength to resist pressure from within. I prefer that no part shall be

stretched more than two-fifths as much as would cause permanent sensible enlargement. Hard steel is a suitable material for the outer parts and mild steel for the inner. However, I find it convenient sometimes to use wrought-iron, bronze, or soft steel or steel hardened in oil for the inside, and various qualities of cast iron for the center and outside parts; or sometimes I use cast-iron for the center part or parts with steel outside and wrought-iron or brass inside.

I do not confine myself to any of the precise arrangements of materials described, but I arrange any suitable materials so that their extensibility within the elastic limit shall be greatest inside the gun and least outside. The elasticity of the same metal, especially if it is steel, may be modified by various processes of hardening and annealing, &c. The strengthening is not necessary the whole length of the gun.

The accompanying drawing is a section of a four and three fourths inch gun I have made. A is a tube of mild steel, surrounded by B, a tube of harder steel, over so much of its length as is necessary to resist the pressure of the gas of the gunpowder where great. Before being put on, the inner diameter of B was about one two hundredths part of an inch less than the outer diameter of A, because the inside of B could stretch without risk of injury so much more than the outside of A would be stretched when the inside of A was extended so far as consistent with perfect safety.

I claim—

The manufacture of cannon composed of two or more tubes having successively-decreasing amounts of extensibility within the extensible limit, (the inner tube having the greatest amount,) when these tubes are put together with initial tension, substantially in the manner and for the purpose described.

T. A. BLAKELY.

Witnesses:

R. A. BROOMAN,  
I. C. MEWBURN,  
Both of 166 Fleet Street, London.